

Nov. 7, 1944.

R. A. HOLBROOK ET AL

2,362,378

FILLING MIXTURE FOR SHOE BOTTOMS

Filed May 23, 1940



INVENTORS  
Ralph A. Holbrook  
Willis G. Hooker  
By *W. J. Smith*  
ATTORNEY

## UNITED STATES PATENT OFFICE

2,362,378

## FILLING MIXTURE FOR SHOE BOTTOMS

Ralph A. Holbrook, Beacon Falls, and Willis O. Hooker, Shelton, Conn., assignors to The Sponge Rubber Products Company, Shelton, Conn., a corporation of Connecticut

Application May 23, 1940, Serial No. 336,762

5 Claims. (Cl. 260—755)

This invention relates to mixtures of substances forming a spreadable mass of material particularly suited for filling the cavity between inner-sole and outersole of a shoe during fabrication or repair. The invention further relates to preferred methods for making the mixture and applying it to the shoe bottom.

Characteristics desirable in mixtures for this purpose include; ability to be smeared thinly over the inverted innersole in the manner of a plastic; ability to "flow" sufficiently under heat and pressure to become molded into full conformity with the boundaries of the cavity; ability to set quickly and without shrinking or cracking; ability to form, when set, a tough, flexible and somewhat resilient layer separating the innersole from the outersole and which shall be proof against creeping and bunching when the shoe is being worn; and freedom from ingredients which can injure either the leather or other materials of the shoe, or the foot of the wearer. It is also desirable that a shoe bottom filling material shall be non-absorbent and waterproof, also that it be able to "breathe" as does the porous leather soles between which it is sandwiched in the shoe bottom. It is further desirable that the mixture shall be inexpensive, which end can best be attained by the use of by-products or reclaimed materials as ingredients.

Former attempts to produce a shoe bottom filling material having the characteristics enumerated have met with serious obstacles. These obstacles have resulted in poor spreading and molding quality, or slow unsatisfactory setting performance of the attempted mixtures, or lack of uniformly distributed coherence, adherence and porosity of the filling in the shoe bottom with resultant creeping and bunching of the filling material when the shoe is in use.

Formerly proposed use of liquid rubber dispersion as a flowable binder mixed with filler bodies comprising ground cork or equally solid particles of other substances has required time wasting waits until the liquid in the rubber dispersion evaporates and permits "setting" of the mixture after its application to the shoe. Also the formerly proposed use of small particles having a solid body character comprising the filler ingredient of the mixture has necessitated the addition of special agents among the ingredients of the mixture to effect an "opening" or porosity thereof in order that air may be admitted to the interior of the mass and aid in the evaporation of its liquid content. This "open" character of the mixture is further needed to help maintain

uniform distribution of the binder throughout the mass after the mixture has been smeared, spread or wiped into its filling position in the shoe bottom, and to prevent balling or rolling up of the material in the course of spreading it into a thin cavity filling layer.

The present discovery teaches that a satisfactory self-opening quality may be imparted to a spreadable mixture of the character concerned by the use of filler bodies or particles composed of ragged membranous scraps or fragments of tough, flexible and preferably resilient substances having the distinctive physical property of possessing a minutely intersticed, creviced or pouched structure. While ground-up particles of natural sponge or artificial cellulose sponge might serve some of the purposes of the ragged membranous scraps referred to, particularly good success has resulted from the use as filler bodies of tiny particles of vulcanized rubber intersticed or minutely creviced or pouched because made up of an attenuated network of thin, tough, elastic, conjoined, curved, membranous walls preferably having their free edges lacineated and shaped to present minute retentive or hook-like protuberances. In particles of such structural nature the projecting of a fragmentary portion of one wall away from the surface of a conjoined wall in itself forms a retentive protuberance even where the wall edges themselves are smooth. Curling of the free marginal edge portions of the walls also forms retentive elements. If the membranous walls of such a particle are perforate, this also will add to the mass opening effectiveness of the improved type of filler body. The present discovery further teaches that filler bodies having the physical properties mentioned may be produced by disrupting, distorting, and irregularly tearing apart vulcanized cellular rubber stock or articles made therefrom, and hence such by-products or scrap pieces of sponge rubber may form a source of supply of this desirable kind of filler particles. Thus when ordinary sponge rubber is ground up into fine particles, the cell-surrounding membranous walls of the sponge rubber structure tear irregularly and curl over and some of them may also become perforate. With filler bodies of the kind above indicated, various binders may be used. Particular success has attended the mixing with such filler bodies of granules of a waxy vegetable substance softened and made adherent by wetting the granules with a mineral oil. Specifically the waxy substance may be a resin, or rosin, while the oil may be paraffin oil. Variations from these in-

dicated ingredients are mentioned hereinafter. Further particulars as to the qualities and reactions of such a mixture and as to the ways of compounding it and applying it as a filling to a shoe bottom cavity are also hereinafter given with particular reference to the accompanying sheet of drawings wherein:

Fig. 1 shows an inverted partially assembled shoe with a filling material embodying these improvements being applied to the bottom thereof.

Fig. 2 shows a microscopically enlarged fragmentary view of a single particle of the improved filler body.

Figs. 3 to 8, inclusive, are fragmentary views drawn on a still further enlarged scale taken in section respectively on the planes 3—3, 4—4, 5—5, 6—6, 7—7, and 8—8, in Fig. 2, looking in the direction of the arrows.

Figs. 9 and 10 are correspondingly enlarged fragmentary views taken in section respectively on the planes 9—9 and 10—10 in Fig. 3.

Fig. 11 is an enlarged fragmentary view taken in section on the plane 11—11 in Fig. 2 looking in the direction of the arrows and indicates the corresponding interlocking parts of a neighboring filler particle.

Fig. 12 shows on the same scale as does Fig. 2 a fragmentary portion of a single filler particle carrying retained thereagainst granules of a binder substance.

The physical characteristics of the improved filler particle structure are evident from the microscopically enlarged views thereof shown in Figs. 2 to 10 inclusive. In the case of particles of ground up or shredded vulcanized cellular rubber stock whose membranous walls have been torn apart in the grinding process, the tearing action leaves certain of the flexible and elastic membranous walls 9 with serrated or rough edges of hook-like shape forming retentive protuberances 10. The curved nature of the marginal portions of the walls also gives rise to further protuberances 11 some of which may also be of hook-like nature. Also resulting from the irregular tearing apart of the curved membranous walls encompassing the interior cells of the original vulcanized sponge rubber stock are apertures 12 which may be bordered by wall edges shaped to form retentive protuberance 13. It will be observed that the projection of a fragmentary portion 14 of one wall away from the surface 15 of a conjoined wall also forms in effect a retentive protuberance.

While operations of a nature which tear apart the sponge rubber, commonly referred to in the art as "grinding," have been found effectively to produce particles having these characteristics, some such characteristics will result from operations of a nature which cut the sponge rubber into small particles. In either of these methods of dividing the original sponge rubber into particles having the novel characteristics described, it has been found to be of advantage that the resulting particles shall vary in size, in order that a certain proportion of the finest particles or crumbs shall be small enough to enter and occupy voids which would be left by the larger particles alone and thus prevent uneven distribution of such voids.

The various forms of retentive protuberances perform several functions of importance to the desirable performance of the improved filling mixture. First they effect a yieldable mechanical interlocking with crevices and/or pouches formed by similar protuberances, as 11' in Fig. 11, on

neighboring like filler particles. They add to the plastic nature of the physical mixture by virtue of their relative weakness and ability to yield and distort in a manner to fit into available spaces 5 when the mixture is compacted or squeezed together in the act of smearing it against the shoe bottom. Because of their resilient nature, these tiny protuberances further tend to spring back somewhat after being pressed or matted together 10 or otherwise distorted and thus automatically promote an opening action throughout the mass of filling mixture which gives better access for air to enter and aid in the rapid and uniform setting of the binder. They furnish mechanical holding means for relatively much smaller solid granules 15 of a resinous binder substance or rosin.

The mechanical interlocking of the retentive protuberances on neighboring contacting tiny filler particles and the retention of the still 20 smaller grains or granules 16 of oil-softened rosin or other binder material well distributed over the irregular surfaces of the filler particles as shown in Fig. 12, is aided by the presence of irregular apertures 12 in the membranous walls. Some of the protuberances 10 or 11 and some of the granules 16 of the binder substance are certain 25 to enter and become separably lodged in these apertures. Thus a plurality of the binder solids are lodged shiftably against and separably retained by the disrupted creviced and pouched cellular walls of a single filler fragment in scattered and spaced relation.

With this understanding of the valuable properties of the distinctive intersticed creviced and 30 pouched structural make-up of each tiny filler particle, whose over-all dimension may be  $\frac{1}{16}$  inch or less and still contain all of the minute intersticed and lacinated detail illustrated in Fig. 2, it will be appreciated that a radically different 35 performance and reactance may be expected of a mixture containing filler body particles of this nature than is the performance and reactance of a mixture in which only solid particles of ground rubber, ground cork, or other equally solid substances are used.

In preferred practice, and subject to variations as desired, 100 pounds of vulcanized sponge rubber scrap in the form of dry particles, sifted to 35 eliminate particles which will not pass through a  $\frac{3}{32}$  " screen, are dumped into a mixer, together with 100 pounds of pulverized rosin and 5  $\frac{1}{2}$  quarts of a thin paraffin oil. The whole is tumbled or otherwise thoroughly mixed together causing the rosin to be thoroughly wetted by the oil and 40 causing the oil to coat all surfaces of the rubber filler particles. The intersticed creviced and pouched nature of the filler particles presents in a given cubical dimension of space much more surface area receptive to coating by the oil, and receptive to a distribution thereover of the granules of rosin, than would be possible to solid filler particles of any substance. This therefore makes for more intimate, uniform and thorough distribution of the oil softened rosin granules in relation to the filler bodies and produces more ready response of the whole binder content to the application of heat when the mixture 17 is troweled into the shoe bottom cavity by means of the heated metallic blade of a hand tool 18, or by 45 a hot presser roller or other heated pressing means. With or without heating, the oil promotes adherence of the binder granules to the walls of the sponge rubber filler fragments. Sufficient resinous binder is used to bond the 50 sponge rubber particles at their points of con-

tact preferably without filling up or badly clogging the desirable interstices throughout the mixture thereby to preserve the open and workable consistency of the mass. Sufficient oil is used to coat the sponge rubber particles and wet the resinous binder.

In place of smearing a bulk mass of our improved filler mixture against the bottom surface of the inner sole of the inverted shoe, a preshaped sole-like blank may be cut or stamped out of a sheet of stock of suitable thickness composed of our improved mixture of materials, such blank fitting nicely the cavity in the shoe bottom which is to be filled. Such stock may be prepared for sale in suitable flat or rolled sheet form by warming a mass of the mixture which has hereinbefore been described until the waxy granules melt and spread evenly and throughout between the rubber filler particles. In this condition the plastic-like mass is rolled or pressed into sheet form and allowed to cool and set whereupon the resolidification of the waxy filler substance enables the mixture flexibly to retain a sheet form of predetermined thickness which thereupon may be sold either flat or in rolls for the intended purpose of stamping out from it the sole-shaped blanks for use as shoe fillers. This then requires only pressure and heat but no troweling or like hand-tool operation to apply to the shoe.

Limited departure from the substances which have herein been proposed for binder may be resorted to without losing all of the advantages which arise from the nature of the filler particles concerned. Waxy binders to serve the purpose of granules of rosin may be selected from a group of mineral substances and softening or lubricative oils may be chosen from a group of vegetable liquids. Castor oil may serve a softening or lubricative purpose. Both the sticky or solidifiable substance and the softening or lubricative substance may be such as will assume a liquid form at ordinary room temperatures. Shellac used as a liquid substitute for solid rosin will be found to have valuable properties. Where both binder substances are liquid no preheating to make the mixture spreadable or workable will be required.

With the foregoing specifications as guide to aid in availing of the present improvements in shoe filler mixtures, it will be understood that many of the advantages thereof may be obtained by the use of well known substitutes and equivalents for substances actually named, wherefore the appended claims will be understood to cover and apply to all such substitutes and equivalents as fairly come within their terms.

It will be understood that there are many uses for our improved composition other than that of filling shoe bottoms. Among these there may be mentioned the calking of seams and crevices in marine and building structures to make weather-proof and the filling of various cavities in assembled articles whose use involves the flexing or stretching of the walls thereof.

We claim:

1. A shoe filler comprising particles of shredded sponge rubber mixed with sufficient resinous binder yieldably to bond the sponge rubber particles at only their points of contact, and an oil in quantity sufficient to coat the sponge rubber particles and wet the resinous binder.
2. A shoe bottom filler mixture including, flexible elastic filler fragments composed of disrupted membranous walls of cellular vulcanized rubber, minute binder solids comprising granules of resinous binder so tiny that a plurality of said granules are shiftably lodged against and separably retained by said disrupted cellular walls of a single filler fragment in scattered relation over the surface of said walls, and a sufficient quantity of an oil to coat the exposed surfaces of said rubber filler fragments and to wet said granules of resinous binder for causing the latter to soften and become more sticky thereby to promote adherence of said granules to said rubber walls in their said scattered relation.
3. A shoe bottom filler mixture including, raggedly contoured flexible elastic filler fragments composed of conjoined disrupted membranous walls of cellular vulcanized rubber, minute sticky binder solids comprising granules of resin so tiny that a plurality of said granules are shiftably lodged against and separably retained by the contours of said disrupted cellular walls of a single filler fragment in scattered relation over the surface of said walls, and a sufficient quantity of an oil to coat all exposed surfaces of said rubber filler fragments and to wet said granules of resin for causing the latter to soften and become more sticky thereby to promote adherence of said granules to said rubber walls in their said scattered relation.
4. A shoe bottom filler mixture including, raggedly contoured flexible elastic filler fragments sufficiently small to pass through screening apertures of the order of three thirty-seconds of an inch in breadth composed of conjoined disrupted membranous walls of cellular vulcanized rubber, minute sticky binder solids comprising granules of resin so tiny that a plurality of said granules are shiftably lodged against and separably retained by the contours of said disrupted cellular walls of a single filler fragment in scattered relation over the surface of said walls, and a sufficient quantity of an oil to coat all exposed surfaces of said rubber filler fragments and to wet said granules of resin for causing the latter to soften and become more sticky thereby to promote adherence of said granules to said rubber walls in their said scattered relation.
5. A shoe bottom filler mixture including in an exemplary batch approximately one hundred pounds of free minutely intersticed filler particles composed of finely fragmented cellular rubber stock, approximately one hundred pounds of pulverized rosin, and approximately five and one half quarts of thin paraffin oil.